

## UNITED STATES PATENT OFFICE

MAURICE O. EDMISTON, OF ST. LOUIS, MISSOURI

## LUBRICANT

No Drawing.

Application filed March 30, 1927. Serial No. 179,716.

This invention relates to improvements in lubricants and method of compounding the same, and refers more particularly to a lubricating composition having for its components a mineral oil, a fatty acid or fatty acids, and a neutralizing agent, such as a caustic blended or compounded with the mineral oil, and acid with a vehicle such as substantially anhydrous glycerin, the caustic alkali or other neutralizing agent being present in an amount sufficient to completely neutralize the acids present.

It is recognized as common practice to add fixed oils, such as animal or vegetable oils, or fats to mineral oils to form a lubricating compound and also it is well known in the art to form a soap in a lubricating compound containing fixed oils by the use of an alkali. In the compounding of the present lubricant, to a mineral oil is added a fatty acid or fatty acids, and to this mixture is combined with an alkali dissolved in a solvent. The manner of combining the fatty acid or acids, the alkali solution and the mineral oil may be accomplished in any suitable manner; either the fatty acids combined with the alkali solution and the resultant mixture supplied to the mineral oil, or the fatty acids added to the mineral oil, 30 and the alkali solution combined therewith.

The mixture, however made, is preferably brought to a temperature sufficient to eliminate any moisture present. Moisture or water has the objective tendency of separating the constituents of the compound. The neutral compound resulting from the mixture of acid and alkali remains liquid and in solution with the mineral oil as contrasted with a lubricant in which the alkali is combined in an aqueous solution and the water driven off. The latter case produces a relatively hard soap unsoluble in the mineral oil while in the former case the soap remains liquid.

The function of the glycerin is primarily as a vehicle to carry the alkali into the mixture to neutralize the fatty acids present. The glycerin, in the amount used, also has no substantial effect upon the viscosity of the oil. Furthermore, the glycerin is miscible

with all of the ingredients, and consequently will not have the effect of an aqueous solution, in bringing about separation or ropiness in the compound.

Among the fatty acids which are adaptable to this purpose are practically all of the range of fatty acids, including butyric, caproic, caprylic, capric, linoleic, myristic, ricinoleic, palmitic, stearic, and oleic. Among the above, which are particularly adapted to this purpose, are oleic and stearic acids. The alkali materials used to neutralize the fatty acids in the combination or mixture, are potassium and sodium hydroxides, which are added to the mixture in a solvent such as glycerin.

A further advantage of the use of glycerin as a solvent for the alkali is the fact that the cold test of the oil is not raised and remains substantially the same as the pure mineral oil used in the combination. It is a recognized fact that in the compounding of mineral oils with vegetable or animal oils, the cold test is decidedly effected. Fixed oils, or fats, have a relatively high cold test, which effect the cold test of the mixture when combined with mineral oil, but in the present mixture or compound, the use of glycerin, which has a low cold test, offsets the effect of the high cold test of the fixed oils. The combining of fixed oils and mineral oils is perhaps the present practice, which is somewhat similar to the present invention. Such combinations under the effect of high temperature and in the presence of moisture decompose to form fatty acids, which are objectionable as such, due to their effect upon the metals with which they come in contact, causing pitting and corrosion.

Where a combination of a mineral oil and fixed oils containing fatty acids is used at high temperatures, and in the presence of steam, or moisture, objectionable soap-like deposits accumulate in the passages and metallic soaps and oxides of iron are produced by the corrosion of the metal, also free carbon accumulates and all of these objectionable ingredients, together with deposits of solid matter from the water, produce diffi-

culties in the effective use of such a lubricant, this impairing the efficient operation of the machine.

The present invention provides a lubricant 5 in which the fatty acids are neutralized with the alkali dissolved in the glycerin, and any soap formed has the effect of retaining the mineral oil on the metal surfaces in a thin film, preventing metal to metal contact. 10 This is a decided advantage over the use of straight mineral oil which would be readily washed away due to the tearing action of moisture present.

The metallic oxides, carbonaceous deposits 15 its or mineral deposits from the water, dust or other deleterious material, held together by mineral oil and depositing and accumulating in the cylinders or in the passageways of the engine, are cleaned by the detergent 20 effect of the neutral soap, formed in the combination of the alkali and fatty acids. This soap is kept in a fluid state by the presence of the glycerin.

While the lubricant has been explained 25 particularly in connection with steam engine practice, it is a fact that this combination of mineral oil, a fatty acid, or fatty acids, and an alkali material, dissolved in glycerin is applicable to air compressors, internal 30 combustion engines, including Diesel use. The particular mixture for each practice will vary according to the requirements, that is, in the case of air compressor work somewhat lower viscosities will be necessary 35 with corresponding lower cold tests than in steam engine practice.

As a typical example of a steam cylinder liquid lubricant, a major proportion of Mid-Continent oil of 25 Baumé gravity having 40 a flash point of 545° F. and a fire test of 620° F., a viscosity of 150 Saybolt seconds at 210° F., and a cold test of 35° F., was combined with a minor proportion of a compound made from oleic acid and potassium hydroxide in a solution with glycerin. The compounding of the constituents was done in the following manner: The proportions given are according to a pint of the lubricant. To 409 c. c. of the mineral oil 45 was combined 45 c. c. of the mixture of the fatty acid and alkali dissolved in glycerin. Of this mixture substantially nine-thirteenths was oleic acid and four-thirteenths glycerin, and potassium hydroxide; the potassium hydroxide being soluble in glycerin as about one to two and one-half by weight. Preferably the alkali hydroxide may be incorporated in the glycerine by agitation and the solution then mixed with the fatty acid. 50 The resulting material may then be thoroughly mixed with the mineral oil. After or during the mixing of the ingredients sufficient heat is applied to drive off the water present. This mixture was used on a locomotive in actual road tests, and found to be

especially effective in the removal of accumulated deposits referred to heretofore. The resistance of this lubricant to the action of moisture rendered it especially economical, it being found during the road tests that considerably less oil was used than the regular oils heretofore used. 70

The present invention contemplates the use of fatty acids in place of fixed oils or fats, or neutral glycerides containing fatty acids. This permits accurately controlling the neutralization of the fatty acids present, and does not require the presence of an excess of alkali to take care of the acids as they are formed. 75

The invention also contemplates any method of compounding mineral oils and fatty acids with alkali dissolved in glycerin, and furthermore the use of alkali in glycerin when combined with mineral oils, and fixed oils, or fats, to neutralize the fatty acids formed by the breaking down or decomposition of the fixed oils or fats. 80

I claim as my invention:

1. A liquid lubricant comprising a substantially water-free mixture of a major proportion of mineral oil and minor proportions of a fatty acid and an alkali metal hydroxide dissolved in glycerin, the hydroxide being in sufficient amount to neutralize the acid and the resultant neutral compound being dissolved in the mineral oil. 90

2. A liquid lubricant comprising a substantially water-free mixture of a major proportion of mineral oil and minor proportions of oleic acid and an alkali metal hydroxide dissolved in glycerin, the hydroxide being in sufficient amount to neutralize the acid and the resultant neutral compound being dissolved in the mineral oil. 100

3. A method for producing a liquid lubricant which comprises mixing with a major proportion of mineral oil minor proportions of a fatty acid and an alkali metal hydroxide dissolved in glycerin, the hydroxide being in sufficient amount to neutralize the acid and forming therewith a neutral compound soluble in the oil, and heating the resultant mixture sufficiently to remove water. 110

MAURICE O. EDMISTON. 115

120

125

130